

Patented Dec. 28, 1926.

1,611,969

# UNITED STATES PATENT OFFICE.

HERMANN WENZL, OF FRANKFORT-ON-THE-MAIN-SUD, GERMANY, ASSIGNOR TO THE FIRM I. G. FARBEINDUSTRIE-AKTIENGESELLSCHAFT, OF FRANKFORT-ON-THE-MAIN, GERMANY.

## PROCESS FOR PRODUCING HIGH-GRADE HALF STUFF.

No Drawing. Application filed July 8, 1926, Serial No. 121,271, and in Germany January 25, 1926.

This invention relates to the production of high-grade half stuff.

The chemical resolution of dishomogeneous raw fibrous substances affords considerable difficulties, as is generally known. For instance up to date no method is known for resolving flax straw, i. e. wastes which remain every year in immense quantities from the flax-harvest, to paper raw-stuff, although their high contents of valuable cellulose and the intactness and long-fibrousness of the flax fiber afford the best prospects for utilizing the said wastes. For instance, Sidney D. Wells and Earl R. Schafer in the preface to their paper on "Chemical Constituents of Flax Straw" in the "Paper Trade Journal", Vol. LXXX, No. 17 of April 23, 1925, page 47 say what follows:—

"These studies indicate that the compounds of the stem of the flax plant known to the textile and allied trades as bast and shive are widely different in their chemical characteristics. The bast seems to consist of relatively pure cellulose adsorbed to which are carbohydrates soluble in hot water or mild alkaline treatment while the shive is composed of cellulose in close combination with pentosans and lignin. A large number of various treatments failed to indicate any that were capable of softening or disintegrating the shive without marked reduction in the tensile strength of the bast," and on page 50 of the conclusions they say: "That chemical methods exist which are capable of pulping the shive without weakening the bast has not yet come to the attention of the writers."

From this up-to-date quotation it appears with absolute certainty that the dishomogeneous composition of many raw fibrous substances, especially of spinning-mill wastes or other similar cellulosic wastes prohibits a chemical resolution by means of the methods hitherto known.

The object of my present invention is to resolve the raw materials referred to without injuring the strength of the fiber or reducing the output to an undesired degree. This object is attained by a novel composition of the resolving liquor, as more fully explained in the following description.

Substituting magnesium or sodium for calcium in the usual digesting liquors of the cellulose manufacture is well known. Kel-

ler has already in the beginning of the 55 seventies of the past century proposed to employ sodium bisulphite, and Graham, British Patent No. 5365/1882, uses neutral sodium sulphite to which subsequently sulphurous acid is added, so that sodium bisulphite is formed in the course of the process which then acts together with sulphite.

In contradistinction to this the present invention is based on the discovery that the composition of the digesting liquor in view 65 of its two components: bisulphite and sulphite, must from the first correspond to a certain relation, and that excellent results are obtained by following the relation

$$XHSO_3 : X_2SO_3 = 3.0 \text{ to } 3.5 \text{ parts : 1 part.} \quad 70$$

Owing to the reduced solubility of the sulphites and bisulphites of the earth-alkali metals, the production of a digesting liquor composed according to the above formula 75 involves, to a certain degree, the use of alkali metal salts, part of which, however, may be replaced by sulphites or bisulphites of earth-alkali metals respectively, care being taken that the above-mentioned relation 80 of the components be not considerably altered.

Furthermore certain neutral salts are to be added to the digesting liquor above described, the said neutral salts, as it seems, 85 facilitating the extraction of the incrustations without themselves participating in the chemical reaction. Preferably neutral salts may be used which in aqueous solution at elevated temperature are subject to hydrolytic dissociation.

My process is, by way of example, carried out in the following manner:—

10000 kgs. of spinning-mill wastes (flax straw) are mixed in an acid-proof rotary 95 digester with 35000 liters of a solution containing 1800 kgs. of sodium-bisulphite, 540 kgs. of sodium sulphite, and 100 kgs. of magnesium chloride. The digester is closed and, under continuous revolution, left for half an hour without heating. A neutral alkali metal salt as alkali sulphate may be added instead of or in addition to magnesium chloride.

Hereupon it is slowly heated by live 105 steam up to 110° C. and left at this temperature for about 1 hour. After this time the temperature is gradually raised to 145°—

150° C., and after 10 hours the liquid is expelled under pressure; the digested material is several times washed with water and hereafter further treated in the usual 5 way. In this manner a pure half stuff is obtained which is easily bleachable to a pure white and possesses a most satisfactory strength.

10 The invention is also applicable to the treatment of manila, hemp, jute waste and the like, provided that the added neutral salts and the concentration of the digesting liquid are adapted to the material just treated; straw of grain may also be subjected to pulping according to my invention.

15 Instead of immediately treating the fiber with the digesting liquid, as described in the above example, I may also proceed in the following manner:—The fibrous material is first impregnated with a substantially stronger solution of the same composition as indicated, then the excess of liquid is mechanically separated, and now the material is treated with steam under pressure 20 at elevated temperature, so that the concentration of the impregnating liquid gradually passes over to that of the digesting liquid.

I claim:—

1. The process of producing high-grade 30 half stuff, especially from spinning-mill waste, flax, hemp straw, jute and the like, comprising the digesting of the raw materials at an elevated temperature with an aqueous solution containing one part of a monosulphite to between 3 and 3.5 parts 35 of a bisulphite with the addition of a soluble neutral salt.

2. The process of producing high-grade 40 half stuff, especially from spinning-mill waste, flax, hemp straw, jute and the like, comprising the digesting of the raw materials with a concentrated aqueous solution containing one part of a monosulphite to between 3 and 3.5 parts of a bisulphite with the addition of a soluble 45 neutral salt mechanically separating the excess of the solution, and treating the material with steam under pressure at temperatures exceeding 100° C.

50 3. The process of producing high-grade half stuff, especially from spinning-mill waste, flax, hemp straw, jute and the like, comprising the digesting of the raw materials at an elevated temperature with an aqueous solution containing one part of a monosulphite to between 3 and 3.5 parts 55 of a bisulphite with the addition of a soluble neutral salt subject to hydrolytic dissociation in aqueous solution at elevated temperature.

60 4. The process of producing high-grade half stuff, especially from spinning-mill

waste, flax, hemp straw, jute and the like, comprising the digesting of the raw materials with a concentrated aqueous solution 65 containing one part of a monosulphite to between 3 and 3.5 parts of a bisulphite with the addition of a soluble neutral salt subject to hydrolytic dissociation in aqueous solution at elevated temperature, mechanically 70 separating the excess of the solution, and treating the material with steam under pressure at temperatures exceeding 100° C.

5. The process of producing high-grade 75 half stuff, especially from spinning-mill waste, flax, hemp straw, jute and the like, comprising the digesting of the raw materials at an elevated temperature with an aqueous solution containing one part of sodium sulphite to between 3 and 3.5 parts 80 of sodium bisulphite, with the addition of a further neutral soluble alkali salt and magnesium chloride.

6. The process of producing high-grade 85 half stuff, especially from spinning-mill waste, flax, hemp straw, jute and the like, comprising the digesting of the raw materials at an elevated temperature with an aqueous solution containing one part of a monosulphite to between 3 and 3.5 parts 90 of a bisulphite with the addition of an alkali sulphate and magnesium chloride.

7. The process of producing high-grade 95 half stuff, especially from spinning-mill waste, flax, hemp straw, jute and the like, comprising the digesting of the raw materials at an elevated temperature with an aqueous solution containing one part of sodium sulphite to between 3 and 3.5 parts 100 of sodium bisulphite, with the addition of an alkali sulphate and magnesium chloride.

8. The process of producing high-grade 105 half stuff, especially from spinning-mill waste, flax, hemp straw, jute and the like, comprising the digesting of the raw materials at an elevated temperature with an aqueous solution containing one part of a monosulphite to between 3 and 3.5 parts of a bisulphite with the addition of magnesium chloride.

110 9. The process of producing high-grade half stuff, especially from spinning-mill waste, flax, hemp straw, jute and the like, comprising the digesting of the raw materials with a concentrated aqueous solution 115 containing one part of a monosulphite to between 3 and 3.5 parts of a bisulphite with the addition of magnesium chloride, mechanically separating the excess of the solution, and treating the material with steam 120 under pressure at temperatures exceeding 100° C.

In testimony whereof I affix my signature.  
HERMANN WENZL.